

March 27, 1951

W. K. A. KOERBER ET AL

2,546,642

LIGHT-SENSITIVE PHOTOGRAPHIC EMULSION

Filed April 28, 1947



A----- = Mercapto - butyric acid - p - toluide

B----- = 2 - p - dimethylamino - styryl - 4 - methyl -  
thiazole ethiodide

C----- = Mercapto - butyric acid - p - toluide + 2 - p -  
dimethylamino - styryl - 4 - methyl - thiazole  
ethiodide.

*Inventors*  
WILLEM KAREL ANTOON KOERBER  
DÉSIRÉ MARIA ALOYSIUS VAN GOETHEM  
By *Richard [Signature]*  
Agent

## UNITED STATES PATENT OFFICE

2,546,642

LIGHT-SENSITIVE PHOTOGRAPHIC  
EMULSION

Willem Karel Antoon Koerber, Berchem-Antwerp, and Désiré Maria Aloysi Van Goethem, Kontich, Belgium, assignors to Gevaert Photo-Producten N. V., Mortsel-Antwerp, Belgium, a company of Belgium

Application April 28, 1947, Serial No. 744,522  
In Germany September 5, 1941

Section 1, Public Law 690, August 8, 1946  
Patent expires September 5, 1961

6 Claims. (Cl. 95—7)

1

This invention relates to light-sensitive photographic silver halide emulsions, and more particularly to such emulsions of increased color sensitivity.

The primary object of our invention is to provide an improved light-sensitive photographic silver halide emulsion.

A more specific object is to provide a light-sensitive photographic emulsion having a "supersensitizing" quality. It is known to increase the spectral sensitivity of a photographic emulsion by simultaneously using a sensitizing dyestuff, which is called main sensitizer, and a second sensitizing dyestuff called supersensitizer. For instance, by simultaneously using carbocyanines and pseudocyanines, the general sensitivity of the emulsion is much higher than it would be theoretically by the mere additional action of a sensitizer. In the photographic art, such an increase in spectral sensitivity is known as "supersensitizing."

A still more particularized object is to provide a light-sensitive photographic emulsion containing a supersensitizing combination of a styryl dye and an organic compound of the kind disclosed hereinafter.

Further objects of the present invention are to provide a method of increasing the sensitivity of photographic emulsions sensitized with styryl dyes, a process for sensitizing photographic emulsions with a supersensitizing combination of a styryl dye and said organic compound disclosed further below.

A still further object is to provide a photographic element comprising a support coated with such a supersensitized emulsion.

Other more specific objects will become apparent during the perusal of this specification.

It is known to use styryl compounds for the optical sensitizing of photographic silver halide emulsions.

Though the supersensitizing action is generally obtained by the combined use of two or more dyestuffs, it has already been proposed to accomplish the supersensitizing effect by the use of special cyanine dyestuffs in combination with non-sensitizing organic compounds containing an amino group.

Unexpectedly, we have found that the color sensitivity of photographic emulsions sensitized by means of styryl compounds may be increased

2

to an extraordinary extent by the addition to the emulsion of products corresponding to the following general formula:



10 wherein

Y represents hydrogen or aryl;  
Y' represents aryl or substituted aryl;  
X represents alkyl or hydrogen; and  
X' represents alkyl.

15 The present invention enables the supersensitizing of both silver chloride and silver bromide emulsions sensitized by styryl compounds, improving simultaneously the stability thereof.

As the main sensitizer all styryl dyestuffs may, 20 be used which correspond to the following general formula:



wherein

D represents non-metallic atoms necessary to complete a heterocyclic 5- or 6-membered ring;  
R represents alkyl, aryl or aralkyl;  
X represents halogen or any acid residue; and  
n represents a positive integer:

25 R' represents residues of secondary amines, for instance, 2-p-dimethylamino-styryl-quinoline ethiodide, 2-p-dimethylamino-styryl-benzthiazol methiodide, 2-p-dimethylamino-styryl-beta-naphthothiazole-methiodide, 2-p-dimethylamino-styryl-4-methyl-thiazole ethiodide, 2-p-dimethylamino-styryl-benzoxazole benzyl bromide.

According to the present invention, products capable of increasing the activity of these dyestuffs are, for instance, the following:



Alpha-mercaptop-n-butyric acid naphthyl amide



Alpha-mercaptop-propionic acid p-toluidide



Alpha-mercaptop-iso-valeric acid p-chloroanilide



Alpha-mercaptop-iso-butyric acid p-toluidide

The preparation of these supersensitizers is described in Beckurts and Frederichs, Archiv der Pharmazie 253, page 161.

To carry out the method of the present invention, the main sensitizer and supersensitizer may simultaneously be added to the emulsion; or the coated light-sensitive emulsion already containing the main sensitizer may be bathed in a solution of the supersensitizer; or the non-sensitized emulsion layer may be bathed in a mixture of the two sensitizers. Finally, the supersensitizer may be added to the anti-stress layer or to the barite layer.

The light-sensitive emulsion may be prepared with the help of any binder known in the photographic emulsion technique, e. g., gelatine and vinylpolymers.

The method of our invention is illustrated by the following specific example:

A silver chloride emulsion according to Eder Handbuch III, 5th edition, 1903, page 727, is prepared in the following way:

- (A) 15 g. of sodium chloride,
- 10 g. of citric acid,
- 20 g. of gelatine
- 200 cm.<sup>3</sup> of water;
- (B) 30 g. of silver nitrate,
- 50 cm.<sup>3</sup> of water;
- (C) 20 g. of gelatine,
- 250 cm.<sup>3</sup> of water.

(A) and (C) are melted at 45° C., (C) is added to (B) whilst stirring, and immediately afterwards (A) is added to (B) + (C). Next, 2 cm.<sup>3</sup> of a 0.1% 2-p-dimethylamino-styryl-4-methyl-thiazole ethiodide solution are added and this mixture is allowed to ripen for one hour. Thereupon 4 cm.<sup>3</sup> of an alcoholic solution of a 1% mercaptop-butyric acid-p-toluidide solution are added, and after 15 minutes the emulsion is cast. The sensitivity of this emulsion is illustrated by the accompanying drawing which is self-explanatory.

It will be apparent that while we have described our invention in preferred forms, many changes and modifications may be made without departing from the spirit of the invention defined in the following claims.

We claim:

1. A light-sensitive photographic silver halide emulsion containing as a sensitizer 2-p-dimethylamino-styryl-4-methyl-thiazole ethiodide and as a supersensitizer alpha-mercaptop-iso-butyric acid p-toluidide.

2. Light-sensitive photographic silver halide emulsion containing at least one sensitizing dyestuff corresponding to the general formula:



wherein

D represents the non-metallic atoms necessary to complete a member selected from the group

75

D represents the non-metallic atoms necessary to complete a member selected from the group

consisting of heterocyclic 5-membered and heterocyclic 6-membered rings,

R represents alkyl, aryl, aralkyl,

R' and R'' represent alkyl,

5 X represents a member selected from the group consisting of halogen and an acid residue, and n represents a positive integer,

and as a supersensitizer at least one product of the general formula:



10 wherein

Y' represents aryl,

X represents a monovalent group selected from the group consisting of alkyl and hydrogen, and

20 X' represents an alkyl group.

3. Light-sensitive photographic silver halide emulsion containing at least one sensitizing dyestuff corresponding to the general formula:



25 wherein

D represents the non-metallic atoms necessary to complete a member selected from the group consisting of heterocyclic 5-membered and heterocyclic 6-membered rings,

35 R represents alkyl, aryl, aralkyl,

R' and R'' represent alkyl,

X represents a member selected from the group consisting of halogen and an acid residue, and n represents a positive integer,

40 and as a supersensitizer alpha-mercaptop-n-butyric acid naphthyl amide.

4. Light-sensitive photographic silver halide emulsion containing a sensitizing dyestuff corresponding to the general formula:



45 wherein

D represents the non-metallic atoms necessary to complete a member selected from the group consisting of heterocyclic 5-membered and heterocyclic 6-membered rings,

55 R represents alkyl, aryl, aralkyl,

R' and R'' represent alkyl,

X represents a member selected from the group consisting of halogen and an acid residue, and n represents a positive integer,

60 and as a supersensitizer alpha-mercaptop propionic acid-p-toluidide.

5. Light-sensitive photographic silver halide emulsion containing a sensitizing dyestuff corresponding to the general formula:



70 wherein

D represents the non-metallic atoms necessary to complete a member selected from the group

5

consisting of heterocyclic 5-membered and heterocyclic 6-membered rings,

R represents alkyl, aryl, aralkyl,

R' and R'' represent alkyl,

X represents a member selected from the group consisting of halogen and an acid residue, and n represents a positive integer,

and as a supersensitizer alpha-mercapto-isovaleric acid p-chloroanilide.

6. Light-sensitive photographic silver halide emulsion containing a sensitizing dyestuff corresponding to the general formula:



wherein

D represents the non-metallic atoms necessary to complete a member selected from the group

5

consisting of heterocyclic 5-membered and heterocyclic 6-membered rings,

R represents alkyl, aryl, aralkyl,

R' and R'' represent alkyl,

X represents a member selected from the group consisting of halogen and an acid residue, and n represents a positive integer,

and as a supersensitizer alpha-mercapto isobutyric acid p-toluidide.

WILLEM KAREL ANTOON KOERBER.  
DÉSIRÉ MARIA ALOYSIUS VAN GOETHEM.

6

#### REFERENCES CITED

The following references are of record in the file of this patent:

#### UNITED STATES PATENTS

|    | Number    | Name | Date          |
|----|-----------|------|---------------|
| 20 | 2,075,046 | Mees | Mar. 30, 1937 |